

# UNITED STATES PATENT OFFICE.

NIELS CHRISTIAN FUNDER JENSEN, OF SOUTHALL, ENGLAND.

## PRESERVATION OF METAL AND METALLIC ARTICLES.

1,354,487.

Specification of Letters Patent.

Patented Oct. 5, 1920.

No Drawing.

Application filed April 23, 1919. Serial No. 292,083.

To all whom it may concern:

Be it known that I, NIELS CHRISTIAN FUNDER JENSEN, a subject of the King of Great Britain, residing at Southall, in the county of Middlesex, England, have invented new and useful Improvements Relating to the Preservation of Metals and Metallic Articles, of which the following is a specification.

10 This invention relates to the treatment of metals and metallic articles for preserving them from oxidation or rusting and other influences and has reference to the kind of treatment in which the metal is furnished 15 with a protective adherent film as the result of the application of oil and a high temperature.

According to this invention the metals, metallic articles or the like are dipped or 20 immersed in a bath of ordinary or common lubricating oil having a proportion of paraffin mixed therewith to render the same of a suitable consistency so as to be sufficiently fluid thin or mobile and then drained to 25 draw off superfluous oil deposit. The drained metals or articles are then subjected to heat in an appropriate chamber or oven whereof the temperature is raised to about 300° C. When the surface of the metals or 30 articles assume approximately a grayish color or mat appearance and the moist or wet condition incidental to the oil bath has been removed therefrom the said metals or articles are taken from the heating chamber 35 or oven and dipped or immersed without previous cooling in an oily mixture consisting for example of whale oil and a mineral oil such as ordinary common lubricating oil. Having been allowed to remain for a 40 suitable period of time in the last mentioned oil mixture the metals or articles are removed and drained whereupon the surfaces are cleaned by means of sawdust or equivalent material.

45 In connection with the first immersion of the metals or articles the bath of lubricating oil has been formed to give good results with a 5% admixture of paraffin the said common lubricating oil being thereby rendered 50 of suitable consistency or fluidity and sufficiently thin or mobile for the purpose of the invention, and as regards the second immersion the oily mixture may consist of equal parts of the whale oil and mineral or 55 common lubricating oil.

In working the process the heating cham-

ber or oven may conveniently be provided with a suitable flue for allowing of the escape of any volatile fluids or fumes resulting from the heating and in order to properly observe the progress of the action on the surfaces of the metals or articles under treatment glazed openings or inspection apertures are provided.

The preservative treatment hereinbefore described is adapted for use with metals or articles possessing clean or rustless surfaces and with metals or articles which have been exposed to atmospheric influences and become oxidized it being unnecessary in the latter case to free the said metals or articles of their coating of rust before subjecting them to the aforesaid preservation treatment.

As the result of the treatment according to this invention the surfaces of the metals or articles are coated with a film of adherent preservative which effectually protects the said metals or articles from the oxidizing influences of the atmosphere. It has also been found that the said adherent film acts as an insulator when employing metals or articles so treated in connection with electrical contrivances.

What I claim and desire to secure by Letters Patent of the United States is:—

1. The herein described treatment of metals and metallic articles for preserving the same from oxidation or rusting and other influences consisting in dipping or immersing the said metals or articles in a bath containing ordinary lubricating oil, draining the superfluous oil deposit therefrom, then subjecting the metals or articles to a temperature of about 300° C. until they assume a grayish tint or ash color, then and without previous cooling again dipping or immersing them in an oily mixture removing and draining them and finally subjecting them to a cleansing action.

2. The herein described treatment of metals and metallic articles for preserving the same from oxidation or rusting and other influences consisting in dipping or immersing the said metals or articles in a bath of ordinary or common lubricating oil having a proportion of paraffin mixed therewith, draining off the superfluous oil deposit, then subjecting the oiled and drained metals or articles to a temperature of about 300° C. in an appropriate chamber or oven until the surface of the metals or articles presents a

grayish color or mat appearance and the moist condition is removed, then dipping or immersing the metals or articles without previous cooling in an oily mixture composed of whale oil and mineral or ordinary common lubricating oil, removing the metals or articles, draining same and finally cleaning the surfaces thereof.

3. The herein described treatment of metals and metallic articles for preserving the same from oxidation or rusting and other influences, consisting in dipping or immersing the said metals or articles in a bath of ordinary or common lubricating oil with a 5% admixture of paraffin, draining off the superfluous oil deposit, then subjecting the oiled and drained metals or articles to a temperature of about 300° C. in an appropriate chamber or oven until the surface of the metals or articles presents a grayish color or mat appearance and the moist condition is removed, then dipping or immersing the metals or articles without previous cooling in an oily mixture composed of whale oil and mineral or ordinary common lubricat-

ing oil, removing the metals or articles, draining same, and finally cleaning the surfaces thereof.

4. The herein described treatment of metals and metallic articles for preserving the same from oxidation or rusting and other influences, consisting in dipping or immersing the said metals or articles in a bath of ordinary or common lubricating oil with a 5% admixture of paraffin, draining off the superfluous oil deposit, then subjecting the oiled and drained metals or articles to a temperature of about 300° C. in an appropriate chamber or oven until the surface of the metals or articles presents a grayish color or mat appearance and the moist condition is removed, then dipping or immersing the metal or metals without previous cooling in an oily mixture consisting of equal parts of whale oil and mineral or ordinary lubricating oil, removing the metals or articles, draining same, and finally cleaning the surfaces thereof.

NIELS CHRISTIAN FUNDER JENSEN.